

# UNITED STATES PATENT OFFICE.

AUGUST E. NIENSTADT, OF BENSONHURST, NEW YORK, ASSIGNOR TO SPECIFICATION  
SOAP & OIL CO., INC., OF NEW YORK, N. Y., A CORPORATION OF NEW YORK.

## PAINT AND VARNISH REMOVER.

1,143,130.

Specification of Letters Patent. Patented June 15, 1915.

No Drawing.

Application filed September 25, 1914. Serial No. 863,462.

*To all whom it may concern:*

Be it known that I, AUGUST E. NIENSTADT, a citizen of the United States of America, and a resident of Bensonhurst, county of Kings, and State of New York, have invented certain new and useful Improvements in Paint and Varnish Removers, of which the following is a specification.

10 This invention has reference to a novel paint and varnish remover to be used, for removing paint and varnish, for instance on railroad cars, partitions, doors and other wood works, and all other painted or varnished surfaces.

Paints and varnishes applied to surfaces may be removed by subjecting such surfaces to the treatment of certain solvents. However, railroad cars and certain wood works 20 have vertical walls with painted or varnished surfaces and active solvents known to soften the paint or varnish and take it up are easily flowing. Accordingly the active solvents will not stay on a painted or varnished vertical surface for a sufficient length 25 of time to render possible the removal of the paint or varnish. For this reason such paint and varnish removers contain a vehicle adapted to form with the solvents a semi-liquid or creamy substance. The vehicle increases the consistency or viscosity 30 of the varnish remover. If such a semi-liquid varnish remover is applied to a vertical surface or even a ceiling it will stay thereon and soften and dissolve the varnish 35 so that it may be removed.

Various substances are employed to act as a vehicle for the active solvents but none of them appears to have given entire satisfaction 40 because the substance or substances forming the vehicle have been selected for the purpose of thickening the remover and usually permit of an undesirably quick evaporation of the active solvents. As a consequence the full effect of the active solvents is not attained and the remaining vehicle 45 has no effect on the varnish.

The present invention has for its purpose to produce a paint and varnish remover in 50 which the described defects have been avoided. This has been primarily attained by selecting such substances for the vehicles and such solvents which produce a semi-liquid or creamy paint and varnish remover

and retard the evaporation of the active solvents sufficiently for obtaining their value to a very high degree. Furthermore, one or the other component of the vehicle may act as an auxiliary means for softening the paint or varnish which increases the efficiency of the remover. It is also important that corrosive strongly caustic or acid substances do not form preponderant components of a paint and varnish remover because such substances destroy and discolor 65 the surface of the wood which renders it difficult to apply a new coat of varnish and as rather transparent varnishes with a glazy surface are sometimes used, the discoloration of the surface of the wood implies an 70 unsightly appearance.

In carrying my invention into effect I substantially proceed as follows: First I mix the solvents, absolute methyl alcohol or as it is commonly called wood alcohol, acetone, benzene,  $C_6H_6$ , or as it formerly was called benzol and ammonia water of  $26^{\circ}$  B. Now naphthalene, ammonium stearate and castor-oil are incorporated with the mixture of solvents and the entire mass is gently 80 heated until the naphthalene, ammonium stearate and castor-oil are completely dissolved and the mass forms a solution. The solution is agitated while cooling to disturb the crystallization of the naphthalene. The 85 free ammonia forms with the castor-oil a soft soap which is soluble in the solvents. This castor-oil ammonia soap tends to keep the mixture of ammonium stearate and naphthalene in suspension and keeps the 90 formerly solid substances from separation. The resulting product is a semi-liquid, creamy composition.

The proportions in which the components are used may vary within reasonable limits 95 for various applications according to the composition of the paint and varnish to be removed. Furthermore less body carrier or vehicle is required in winter than in summer. One formula which answers for the 100 removal of the usual varnishes contains substantially the following percentages of components, all parts by weight: About  $7\frac{1}{2}$  parts of absolute methyl alcohol,  $7\frac{1}{2}$  parts of acetone, 15 parts of benzene, and 2 parts of 105 aqueous ammonia of  $26^{\circ}$  B. To these solvents about 4 parts of naphthalene, about 8 parts of ammonium stearate and about 2

parts of castor-oil are added and the mixture is heated until a uniform solution has been obtained.

The solvents employed in the present 5 remover all have a relatively low boiling point. Wood alcohol boils at 64.8° C., acetone at 56.3° C. and benzene at 80.36° C. These temperatures show that the solvents easily evaporate at normal temperature. 10 when spread out. For this reason it is essential to retard the evaporation. The castor-oil soap formed aids in retarding evaporation. The naphthalene,  $C_{10}H_8$ , although a solid substance is a pure hydrocarbon, and 15 therefore tends to act as an auxiliary solvent while giving body to the composition. The ammonium stearate is a salt and as a solid substance gives body to the composition. Thus the novel varnish remover utilizes the 20 dissolving power of the active solvents to a very high degree.

I claim as my invention:

1. A paint and varnish remover constituent ingredients of which are absolute methyl

alcohol, acetone, benzene, some weak aqueous 25 ammonium solution, some castor-oil, and a thickening vehicle adapted to produce a semi-liquid, creamy composition.

2. A paint and varnish remover constituent ingredients of which are absolute methyl 30 alcohol, acetone, benzene, some weak aqueous ammonium solution, and some castor-oil, naphthalene and ammonium stearate as a thickening vehicle for the active solvents.

3. A paint and varnish remover constituent ingredients of which are about  $7\frac{1}{2}$  parts of absolute methyl alcohol, about  $7\frac{1}{2}$  parts of acetone, about 15 parts of benzene, about 2 parts of castor oil, about 2 parts of aqueous ammonium of 26° B., about 4 parts of naphthalene, and 8 parts of ammonium stearate. 40

Signed at New York, N. Y., this 23d day of September, 1914.

AUGUST E. NIENSTADT.

Witnesses:

CHARLOTTE C. KRICHNER,  
IDA E. ROLAND.